

April 9, 1935.

R. E. BURK ET AL

1,997,480

PREPARATION OF MOTOR FUELS

Filed Jan. 21, 1931



INVENTORS

Robert E. Burk and  
BY Everett C. Hughes.

Fay Oberlin & Fay  
ATTORNEYS.

## UNITED STATES PATENT OFFICE

1,997,480

## PREPARATION OF MOTOR FUELS

Robert E. Burk and Everett C. Hughes, Cleveland,  
Ohio, assignors to The Standard Oil Company,  
Cleveland, Ohio, a corporation of Ohio

Application January 21, 1931, Serial No. 510,323

3 Claims. (Cl. 196—65)

This invention relates to the preparation of motor fuels, and more particularly fuels feasible for usage under load or compression conditions. In customary gasoline, for instance as produced by straight distillation from crude petroleum of Mid-Continent type, there is an objectionable tendency to develop "knocking" in conditions of high compression or load. A fuel having the otherwise good properties of gasoline while avoiding such tendencies, without compelling recourse to introduction of foreign materials, is accordingly highly important and fundamentally desirable.

To the accomplishment of the foregoing and related ends the invention, then, comprises the features hereinafter fully described and particularly pointed out in the claims, the following description and the annexed drawing setting forth in detail certain illustrative embodiments of the invention, these being indicative, however, of but a few of the various ways in which the principle of the invention may be employed.

In said annexed drawing:

The sole figure is a diagrammatic representation of an embodiment of the process, on the order of a flow-sheet.

In accordance with the present invention, gasolines having knocking constituents, such as ordinary or straight run gasoline, is subjected to conditions of temperature and re-action making fundamental changes in the properties relative to knock. We subject such gasoline to the action of heat, in the presence of oxygen, at temperatures lying in the cracking range, for instance, between 840° F.—1300° F. in general. With the gasoline or naphtha vapor, oxygen conveniently in the form of air, is provided in proportions, for instance, of a range of  $\frac{1}{2}$  up to 5 of air to 1 volume of naphtha vapor. High pressures are not necessary and 100 pounds per square inch need not be exceeded. In fact ordinarily a relatively low pressure is best, just enough to secure a desirable through-put rate. The heating time may vary, depending somewhat upon the temperature, and may range for instance between 0.075 to 1 second.

As an example: A straight run gasoline of initial B. P. 116° F., 5 percent off at 158° F., 28 percent off at 212° F., 35 percent off at 221° F., 75 percent off at 284° F., and 97 percent off at 356° F., with end point 368° F., was passed through a heating zone of temperature of 930° F.—1112° F., together with about  $2\frac{1}{2}$  volumes of air to each volume of naphtha vapor, and under pressure just sufficient for good through-put, the heating time being between 0.2 and 0.5 seconds. The

condensate recovered showed little change in end point, but whereas the original material had knocked violently in a motor with raised compression, the product behaved very satisfactorily.

On such basis, in accordance with our process, it is readily practicable to raise the knock-rating without disarranging the boiling point and gravity conditions. The percent of hydrocarbons soluble in sulphuric acid containing 30 percent P<sub>2</sub>O<sub>5</sub> shows a very material increase. For instance, with a straight run naphtha from Mid-Continent crude, such naphtha having an initial B. P. of about 100° F., and an end point of about 410° F., and 6 percent soluble in sulphuric acid and phosphorus pentoxide mixture, after subjection to the present process there is a percentage of about 24 soluble in the acid mixture, the distillation and gravity constants remaining practically unchanged.

The product may be further treated, if desired, to a finishing lye-wash, as customary.

If still further anti-knock treatment is preferred, the product may be re-passed through the heating and oxygen stage, one or more times. For example, a straight-run naphtha having serious knocking tendency was passed three times through a heating zone at 930° F. with air in 1 to 1 ratio, and 0.7 second time for each pass. The end product was for practical purposes as satisfactory as the specially-compounded type of anti-knock fuels.

In contrast to cracking, it will be noticed that when the same stock naphtha mentioned above was subjected to an ordinary cracking to the same volumetric yield of gasoline the product retained substantially the same knocking tendencies of the original stock.

Other modes of applying the principle of the invention may be employed, change being made as regards the details described, provided the features stated in any of the following claims, or the equivalent of such, be employed.

We therefore particularly point out and distinctly claim as our invention:

1. A process of preparing motor fuel, which comprises heating gasoline vapor fractionated to substantially desired end-point and substantially unmixed with other gasiform hydrocarbons 0.075 to 1 second at a temperature of 840° F.—1300° F. in the presence of  $\frac{1}{2}$  up to 5 volumes of air, without materially changing the end point of the total condensate.

2. A process of preparing motor fuel, which comprises heating gasoline vapor fractionated to substantially desired end-point and substantially

unmixed with other gasiform hydrocarbons 0.2 to 0.5 seconds at a temperature of 900° F.-1112° F. in the presence of  $\frac{1}{2}$  up to 5 volumes of air, without materially changing the end point of the total condensate.

3. A process of preparing motor fuel, which comprises repeatedly subjecting gasoline vapor, fractionated to substantially desired end-point

and substantially unmixed with other gasiform hydrocarbons to a temperature of about 930° F. for about 0.7 second in the presence of about an equal volume of air, without materially changing the end point of the total condensate.

ROBERT E. BURK.  
EVERETT C. HUGHES.